

## UNITED STATES PATENT OFFICE

2,027,829

## METHOD OF CASTING TRANSPARENT FILMS

Edouard M. Kratz, Gary, Ind., assignor, by mesne assignments, to Marbo Products Corporation, Chicago, Ill., a corporation of Delaware

No Drawing. Application November 8, 1933, Serial No. 697,150

6 Claims. (Cl. 18—57)

This invention relates to a method of casting transparent films and more particularly to the use of a relieving or partitioning agent in connection with a carrier web to facilitate the stripping of the transparent sheet material from the carrier web after the material has dried thereon.

In the casting of aqueous solutions of various film forming substances, such as casein, gelatin and the like, I have found it most suitable to use 10 a flexible carrier web as the surface on which to cast the film forming solutions. Practical types of carrier webs are described in my Patent No. 1,727,611 and in my pending application Serial No. 678,307, filed June 29, 1933. It is desirable that the carrier web be plasticized so as to impart to it the required degree of flexibility, since otherwise there is a tendency of the surface of the carrier web to break down after continuous operation. In the absence of a plasticizing 20 agent in the carrier web, after continued operation, cracks form in the surface that are very objectionable.

Also, in the case of carrier webs which are coated with baked drying oils, there is always a small 25 quantity of free oil embodied in the coating material forming the web surface which has a tendency to spew out of the casting surface when the carrier web is subjected to heat during the drying operation. Although the quantity of oil 30 that may be released to the surface is very minute during any one cycle of the drying operation, after repeated continuous drying, the amount of oil which spews to the surface is of sufficient quantity to cause the dried film, formed by casting a 35 solution onto the carrier web, to adhere to the surface of the web.

Where the carrier web is provided with a surface of nitrocellulose containing castor oil as a plasticizing agent, there is likewise a tendency for 40 the castor oil to work to the surface. There is also a tendency of some of the materials which spew from the belt to form a film on the surface of the carrier web that imparts a dull or smoky appearance to the finished sheet of cast material.

45 Where the film solution being cast contains a fatty material, wax or the like in the form of an emulsion, there is a tendency of these materials to migrate or spew out of the semi-dried sheet and be absorbed by the carrier web. This 50 is due to the fact that as the film dries, there is a tendency for the outer surface to case harden and the contraction of the film solution, which in some cases contains as much as 90% water, causes the various emulsified materials or plasticizing agents to spew out onto or migrate into the

surface of the carrier web. After a period of time, the carrier web may become saturated with one or more of these emulsified materials or plasticizing agents, with the result that when the carrier web is passed through a drying chamber, the heat causes the plasticizing agent or emulsified material to spew out against the dried sheet and cause the sheet to stick to the carrier web. 5

It is therefore an object of this invention to provide a method of casting transparent film or sheet materials wherein the stripping of the sheet or film material from the carrier web is facilitated by the use of a relieving or partitioning agent.

It is a further important object of this invention to protect the casting surface of a carrier 15 web by the application thereto of a very thin, uniform, continuous coating of a substance that is inert to the ingredients of the carrier web and also of the film solution that is being cast onto the carrier web. 20

It is a further important object of this invention to provide an improved method of casting transparent sheet or film material onto flexible carrier webs, whereby the sheet or film material may be readily stripped from the surface of the 25 carrier web without marring the polished surface of the carrier web or blemishing the surface of the sheet or film material.

Other and further important objects of this invention will become apparent from the following 30 description and appended claims.

The relieving or partitioning agent that I prefer to apply to the surface of the flexible carrier web is a substance that is inert both to the ingredients of the carrier web and also to the ingredients of the film that is being cast thereon. Among the inert substances that I have found to be satisfactory may be mentioned non-saponifiable substances of a greasy, unctuous character, such as solid or semi-solid hydrocarbons, like 35 petroleum jelly and lanolin, or cholesterol, chlorinated diphenyls, and the like.

Petroleum jelly, however, gives the best results. For this purpose, a white petroleum jelly having a melting point of from 118 to 122° F. and a flash point of from 380 to 390° F. is preferred. In order to assist in the spreading of the petroleum jelly over the surface of the carrier web, the petroleum jelly is dissolved in a comparatively low boiling hydrocarbon, such as solvent naphtha, 45 petroleum ether, or the like, so that the solution will dry out very rapidly and leave behind a very thin film of petroleum jelly over the surface of the carrier web. 50

The peculiar property of naphtha of "wetting 55

"out" and spreading rapidly makes it very desirable as a solvent or diluting agent for the petroleum jelly. Other hydrocarbons, such as benzol, are not so well adapted for this purpose because of the tendency of the petroleum jelly to coalesce and contract on the evaporation of these other hydrocarbons. Thus, while various hydrocarbon solvents of relatively low boiling point may be used, most satisfactory results have 10 thus far been obtained by the use of naphtha.

It might also be possible to use petroleum jellies having higher melting points than above specified, but there is a tendency of the higher melting point petroleum jellies to crystallize and cause the surface of the finished film or sheet material to have a smoky or streaked appearance. Further, it is not desirable to use a lower melting point jelly or oil, since there would be a tendency of the material to come to the surface during 15 the casting of the film solution, and the free oily hydrocarbon floating upon the surface of the film solution would cause a break in the surface tension which would result in holes or pores in the finished film.

Various concentrations of petroleum jelly and 20 naphtha may be employed, but preferably a concentration of from  $\frac{1}{2}$  to  $\frac{3}{4}$  of 1% of petroleum jelly by weight of the solution is employed. The concentration of petroleum jelly in the naphtha 25 solution may be increased or decreased, according to the amount of adhesion desired between the dried film or sheet material and the carrier web.

An excessive amount of petroleum jelly applied 30 to the surface of the carrier web is not desirable, since there is a tendency of the dried film to break loose from the carrier web at some stage prior to the final drying operation. This makes it 35 more difficult to wind the dried film or sheet material on a mechanical winding device.

Furthermore, it is not desirable to have an insufficient amount of petroleum jelly, owing to the 40 tendency to tear the film or sheet material if there is too great an adhesion between the dried film or sheet material and the carrier web. Consequently, the quantity of petroleum jelly in solution in the naphtha can be adjusted to any degree so as to give the proper relief between the dried film or sheet material on the carrier web.

It has been found very difficult to apply a film 45 of petroleum jelly of the desired thickness in continuity to the surface of a carrier web by such mechanical devices as rollers, buffers or other coating apparatus. The solution of petroleum jelly in naphtha can, however, be readily applied to the casting surface of the carrier web by a felt wick, which is permitted to lightly contact the surface of the carrier web. A soft felt wick is employed so as not to scratch or mar the 50 polished surface of the carrier web. The lower end of the wick is kept immersed in the solution of petroleum jelly in naphtha and capillary action is relied upon to bring the solution into contact with the surface of the carrier web. Because of the high degree of volatility of naphtha, the solvent evaporates rapidly and leaves a thin, continuous and uniform coating of petroleum jelly on the casting surface of the carrier web.

Inasmuch as petroleum jelly does not crystallize, it has a tendency to flow out with the naphtha and form a thin film that does not form any streaks or cloudy effect upon the surface of the carrier web. Also, since the petroleum jelly is inert toward the ingredients of the carrier web or of the film or sheet forming solution, the thin

film of petroleum jelly protects the surfaces of both the film or sheet material and of the carrier web.

Where the casting of transparent sheet or film material is carried out as a continuous operation, as disclosed in my Reissue Patent No. 17,854, the solution of petroleum jelly in naphtha is continuously applied to the bare surface of the carrier web after the sheet material has been dried and stripped therefrom and prior to the casting 10 operation. The film of petroleum jelly is thus renewed during each cycle of the film or sheet forming operation.

The thin, transparent sheet or film material herein referred may be such as is described in my Patents Nos. 1,893,172, 1,866,410, 1,847,656 and various copending applications. I do not, however, restrict the present invention to any particular film or sheet forming composition, since my invention has wide applicability in this 20 general field.

The particular advantages of my invention nevertheless are realized in connection with the casting of aqueous solutions of film forming materials on flexible carrier webs. Solutions of this type generally include dispersing or emulsifying agents in the nature of soap for lowering the surface tension of the solution and thus aiding in the spreading of the solution on the carrier surface. The presence of such dispersing or emulsifying agents serves an even more important function along this same line where the sheet forming solution is cast upon a surface having a coating of petroleum jelly, in that they tend to 25 reduce the surface tension and thereby facilitate the spreading of the solution over the greasy surface of the carrier web. This enables the sheet forming solution to be cast into films of uniform 30 thickness and free from pin holes or other 35 blemishes.

As the sheet or film is stripped from the surface of the carrier web, it naturally picks up a minute quantity of the petroleum jelly on its surface. The quantity of petroleum jelly thus adhering to the surface of the film or sheet material is not sufficient to impair the transparency of the film and is not, in fact, visible to the naked eye. The almost microscopic film of petroleum jelly on the surface of the sheet material nevertheless serves a useful function in imparting 40 "slip" to the sheet material. By this is meant the property of the sheet material, when stacked, to be removed sheet by sheet without sticking. It frequently happens that sheets of casein or 45 gelatin composition will not slip readily, either owing to surface characteristics or to the fact that the sheets are charged with static electricity. The presence of even a minute trace of petroleum jelly on the surfaces of the sheet material largely eliminates this tendency of the sheets to stick together and gives them the desired degree of slip.

Where the sheet material is being made in a continuous operation, it is obviously necessary to renew the film of petroleum jelly on the carrier web. This is satisfactorily accomplished by 60 permitting the wick, referred to above, to remain in constant contact with the bare surface of the carrier web as it passes on into the coating or casting machine. Under some circumstances, however, the application of the petroleum jelly 65 to the surface of the carrier web may be interrupted from time to time, as where the amount of petroleum jelly remaining on the web after the stripping operation is still sufficient and does not require renewing.

5 I am aware that numerous details of the process may be varied through a wide range without departing from the principles of this invention, and I, therefore, do not purpose limiting the patent granted hereon otherwise than necessitated by the prior art.

10 I claim as my invention:

15 1. The method of protecting the surface of a carrier web in the casting of transparent films thereon, which comprises coating said surface with a solution of petroleum jelly in a volatile solvent and evaporating the solvent therefrom to leave a uniform thin film of petroleum jelly.

20 2. The method of protecting the surface of a carrier web in the casting of transparent films thereon, which comprises supplying a solution of petroleum jelly to a capillary member, contacting said member with said surface and drying the coated surface.

25 3. In the casting of transparent films on a flexible carrier web, the step of protecting the surface of said carrier web by applying thereto a temporary thin coating of a solution of white petroleum jelly in naphtha and evaporating the naphtha.

4. In a continuous process for the casting of

transparent sheet or film material on an endless flexible carrier web, the step of continuously applying to the bare casting surface of said carrier web a solution of petroleum jelly in a volatile hydrocarbon solvent.

5 5. In a continuous process for the casting of transparent sheet or film material on an endless flexible carrier web, the step of continuously applying to the bare casting surface of said carrier web a solution of petroleum jelly in naphtha in 10 which the petroleum jelly is present in an amount equal to between 0.5 and 0.75% by weight of the solution.

15 6. The method of continuously forming transparent sheets or films which comprises wicking a solution of petroleum jelly dissolved in naphtha onto a casting surface, allowing the naphtha solution to spread out on said surface to fully cover the same, evaporating off the naphtha to leave a thin uniform coating of petroleum jelly 20 on the surface, casting an aqueous film forming solution on the jelly coated surface, drying the solution thereon, stripping the resulting film therefrom and repeating said casting and drying operations.

25 EDOUARD M. KRATZ.